

Aug. 19, 1958

P. TARDIEU

2,848,318

MANUFACTURE OF MANGANESE IN LOW-STACK BLAST FURNACE

Filed July 23, 1957



BY

*Raphael Tardieu*

ATTORNEY

# United States Patent Office

2,848,318

Patented Aug. 19, 1958

1

2,848,318

## MANUFACTURE OF MANGANESE IN LOW-STACK BLAST FURNACE

Pierre Tardieu, Edea, Cameroun, Africa, assignor to Pechiney, Compagnie de Produits Chimiques et Electro-metallurgiques, Paris, France, a corporation of France

Application July 23, 1957, Serial No. 673,657

Claims priority, application France July 31, 1956

5 Claims. (Cl. 75—80)

The present invention, which is the result of applicant's researches, relates to a new process for the manufacture of high grade manganese in a shaft furnace of comparatively low height, commonly called a low-stack blast furnace.

High grade ferromanganese containing up to 80% and, even, 85% manganese is manufactured in blast furnaces, but when such apparatus is used, it is necessary to use ore in lump form, as well as metallurgical coke resistant to crushing.

High grade ferromanganese can also be obtained in an electric furnace, but inasmuch as such a furnace consumes electric power, it cannot be used everywhere.

In contrast, the low-stack blast furnace can operate satisfactorily with various fuels and with agglomerates of powdered ore having a low mechanical strength. It can be installed with a minimum of fixed parts, even in areas where electric power is lacking.

The process which is the object of the present invention, makes it possible to obtain a metal responding to the following analysis:

|                     | Percent      |
|---------------------|--------------|
| Manganese           | 89 to 92     |
| Iron                | 1 to 3       |
| Silicon             | 0.10 to 0.50 |
| Carbon              | 6.5 to 7     |
| Sulfur, phosphorous | Traces       |

In the process according to the invention, there can be used a powdered pyrolusite which has been enriched, for example, by a flotation process and possesses the following composition:

|                                           | Percent  |
|-------------------------------------------|----------|
| Manganese (as MnO <sub>2</sub> )          | 60 to 62 |
| Iron (as Fe <sub>2</sub> O <sub>3</sub> ) | 1 to 1.5 |
| Silica (gangue)                           | 2 to 3   |

This ore is agglomerated into balls by means of an organic binder, for example, manioc.

The reducing agent can be anthracite, wood charcoal, or any kind of coke, preferably with a low iron content. In order to obtain the highest manganese content, there can be used, for example, pitch coke or "pechcoke" having an ash content of 0.5–0.6%.

The blast blown into the low-stack blast furnace can be oxygen, or air containing 45 to 70% oxygen. It is possible to preheat the blast, for example, by using the gas which is evolved at the top of the furnace. However, a cold blast can also be blown.

In a preferred embodiment of the invention, the charge is made up of ore and reducing carbon, without addition of any element designed to form a slag. Hence, the latter can only come from the gangue of the ore or from the ashes of the fuel, and only amounts to some tens of kilograms per ton of manganese produced.

The manganese yield exceeds 70% and, frequently, attains 75 to 80%.

The silica contained in the charge is almost entirely

removed with the gaseous stream, probably as SiO. This represents an advantageous feature of the process according to the invention, and makes possible the production of a high-grade manganese.

In order to illustrate the invention, there is described by way of example only, and without limitation, an embodiment of the new process as carried out in a shaft-furnace of the low-stack blast furnace type. The annexed single figure illustrates a partial, vertical section of such a furnace; the indicated dimensions are those of a low-stack blast furnace and suitable for carrying out the present invention, and are given by way of illustration and not by way of limitation.

The furnace used in carrying out the operation comprises a shaft 1, having a total height of about 7 meters, a diameter of 1 meter at the level of the tuyeres 2, and a working height of 3 meters above the same level. Into this low-stack blast furnace there was introduced a smelting charge having the following composition per ton of metal produced:

|                                      |        |      |
|--------------------------------------|--------|------|
| Pitch coke ("pechcoke")              | kg     | 2300 |
| Pyrolusite balls                     | kg     | 2250 |
| Cold blast with a 50% oxygen content | cu. m. | 4000 |

There was obtained with a manganese yield of 77%, a metal having the following composition:

|           | Percent |
|-----------|---------|
| Manganese | 92      |
| Carbon    | 6.8     |
| Iron      | 1       |
| Silicon   | 0.2     |

There were collected about 50 kilograms slag per ton of metal.

In the case of the usual blast furnaces of industrial size, there is observed an increase in coke consumption with an increase in manganese content; it could not, therefore, be foreseen that in a shaft furnace of the small size used in the process of the present invention, the consumption of coke per produced ton of such-grade Mn would scarcely amount to the minimum consumption obtained in a (high) blast furnace. It is quite certain that by using the process according to the invention in a low-stack blast furnace having a diameter of 2 meters or 2.50 meters at the level of the tuyeres, the fuel consumption decreases enormously.

Moreover, it would have been expected that the manganese losses in the gases would be considerable by reason of the relative volatility of the metal and the low height of the furnace. Hence, it was not foreseeable that such high manganese yields would be obtained, while nearly all the silicon in the charge is removed by volatilization.

The process of the present invention is generally carried out at temperatures within the range of about 1750–2200° C.

The term "cold blast" as used in the specification and claims denotes a blast at ambient or normal temperatures.

The carburized manganese manufactured in a low-stack furnace differs essentially from that manufactured in an electric furnace, and from ferromanganese of the usual blast furnace, by the fact that it is possible to obtain economically a product having a very low content of silicon, sulfur and iron.

The low silicon content is the more remarkable because the process does not require the use of an ore particularly low in silicon. It follows that the manganese carbide produced by a low-stack furnace can have wider application than the ferromanganese obtained in the usual blast furnace or in an electric furnace, or manganese carbide obtained by electrothermic process, especially, where it is important to have a low content of iron and silicon.

## 3

and particularly, in the case of alloys of non-ferrous metals having an aluminum, copper, chromium, nickel, etc. base.

I claim:

1. Process for treating silica-containing manganese ores comprising the steps of: treating a charge of said manganese ore and carbonaceous material in a low-stack blast furnace with a blast of oxygen-enriched air, whereby the ore is reduced to produce a high-grade manganese metal ore of low silicon content, and recovering said manganese metal.

2. The method of smelting a silica-containing manganese ore to produce a high-grade manganese product of low silicon content and containing not less than 89% manganese, comprising the steps of: charging a mixture consisting of the said manganese ore and a carbonaceous reducing material into a low-stack blast furnace; blast-

ing the charge with oxygen-enriched air, whereby the ore is reduced to produce the aforesaid high-grade manganese product, and recovering said manganese product.

3. The process of claim 2, wherein the ore is an enriched manganese concentrate in finely divided state.

4. The process of claim 2, wherein the blast has an oxygen content of 45 to 70%.

5. The process of claim 2, wherein a cold blast is used.

## References Cited in the file of this patent

U. S. Bureau of Mines, Report of Investigations, No. R. I. 3477, "Manganese and Its Alloys" (1939). (47 pages, page 5 relied on.)

UNITED STATES PATENT OFFICE  
CERTIFICATE OF CORRECTION

Patent No. 2,848,318

August 19, 1958

Pierre Tardieu

It is hereby certified that error appears in the printed specification of the above numbered patent requiring correction and that the said Letters Patent should read as corrected below.

Column 2, line 40, for "such-grade" read -- such high-grade --.

Signed and sealed this 28th day of October 1958.

(SEAL)

Attest:

KARL H. AXLINE

Attesting Officer

ROBERT C. WATSON  
Commissioner of Patents